

# UNITED STATES PATENT OFFICE.

ADRIAAN FLORIS VAN HALL, FRITZ BASENAU, AND RICHARD CORNELUS JOHANNUS VAN HAAGEN, OF AMSTERDAM, NETHERLANDS, ASSIGNEES TO THE FIRM OF NAAM-LOOZE VENNOOTSCHAP BRIQUET COMPANY (BRIKET MAATSCHAPPIJ), OF AMSTERDAM, NETHERLANDS.

## FUEL BLOCK OR BRIQUET.

1,114,715.

Specification of Letters Patent.

Patented Oct. 20, 1914.

No Drawing.

Application filed August 5, 1910. Serial No. 575,738.

To all whom it may concern:

Be it known that we, ADRIAAN FLORIS VAN HALL, FRITZ BASENAU, and RICHARD CORNELUS JOHANNUS VAN HAAGEN, subjects of the Queen of the Netherlands, residing at Amsterdam, Netherlands, have invented certain new and useful Improvements Relating to Fuel Blocks or Briquets, of which the following is a specification.

10 Many attempts have been made to convert coal or coal-slack, anthracite or anthracite-slack and coke or coke-breeze into blocks or briquets by means of liquid fuel, but for attaining the desired object, it was found necessary, to employ a binding substance and in addition to sulfurize the liquid hydrocarbons or to first convert the liquid hydrocarbons into a more or less solid form, for instance by saponification, and then to 20 mix them with coal to obtain a product resembling briquets. It has also been attempted to convert coal and petroleum residue or wood and said residue or peat and said residue into a solid form, but without 25 any practical success.

According to the present invention, a mixture of coal and coal-slack or waste or anthracite and anthracite-slack or waste or coke and coke-breeze, wood or ligneous waste or peat and other combustible matter on the one hand, and petroleum, or petroleum residue or tar oil, or gas oil or other mineral oils or waste oils, on the other hand, may by a mere mechanical treatment of the 30 said solid carbonaceous and liquid hydrocarbonaceous materials, be brought into such a physical condition, that the mixture can be converted into a solid form by pressure. Moreover, the whole process may be performed in the cold or at ordinary temperature. If desired, a binding substance or other admixtures may be employed at the same time, but the binding substance alone is not capable of bringing a mixture of solid 35 and liquid fuel into a condition in which it can be formed into solid blocks or briquets. By this we mean that where in said process the hydrocarbonaceous liquid or a part of it has to some degree a binding property this 40 property is not the one relied upon to bring out the ultimate cohesion in the briquet; but on the contrary for the purposes of that cohesion the essential characteristic is the continued intense mechanical working to

which the solid and liquid fuels must be 55 subjected in order to bring about the results aimed at by us.

The details of procedure may be as follows:—The solid and liquid combustible materials are mixed together in suitable proportions by means of a mixing machine. The proportions depend on the nature of the raw materials and on the calorific value, which is to be attained. For instance petroleum residue equal to 10 to 40 per cent. of 60 the total weight may be employed, according to the nature of the solid fuel and the purpose for which the product is to be used. A solid fuel, for instance anthracite, is of course manifestly incapable of entering into 65 a coherent unit with other particles of anthracite in the absence of a binder. Similarly the petroleum residue or liquid fuel, which in itself is incapable of acting as a binder for the particles of anthracite, will 70 not by itself be capable of forming or existing as a solid unit. The underlying discovery of this application is that such solid and liquid fuels having what may be called these negative qualities, will, when treated in a 75 certain manner, result in the production of a relatively dry, plastic substance capable of forming homogeneous, coherent, solid units. The means employed to bring about this condition is the kneading machine above described, in which the solid and liquid particles are subjected to repeated or continued 80 mechanical treatment until the desired condition is attained. Whether the transformation of the physical properties of the 85 respective materials depends upon chemical or mechanical principles, or both, has not yet been definitely ascertained. The fact remains, however, that we are the first to have combined these solid and liquid fuels into 90 coherent, stable, solid masses without the use of binders. It is apparent that as the kneading process goes forward, the solid fuel will be, to a certain extent, broken into 95 fine fragments, and that the larger particles of the solid fuel will be subjected to the 100 repeated rolling or kneading motion, so that as the mass becomes drier, it will finally be discharged from the machines in the form of coarsely granular conglomerate and relatively dry particles. The precise degree of dryness will, of course, depend upon the 105 duration of the mechanical kneading proc-

ess. Under usual conditions the granular conglomerate particles are in a condition in which they will not become pasted together during transportation, but in which they can be poured from a container like peas from a jar. These relatively dry coarse particles, when pressed by hand or in a suitable mold, will, however, because of their plastic condition, readily unite into a coherent, homogeneous mass of permanent shape. After the said two different types of fuel have been uniformly mixed, the mixture is subjected to a mechanical treatment by rollers, grind-stones or kneading machines, until the material has assumed a drier and a plastic or viscous condition, after which the material is ready for being pressed and may be pressed into the desired shape of blocks or briquets.

Where herein above we have referred to liquid hydrocarbonaceous materials or liquid combustible materials, we mean to refer to fuels which are liquid during the kneading operation as carried out in the machines above referred to rather than to physical characteristics of said fuel under conditions other than those that are present in the kneading machines. The product thus obtained is suitable for storage and for transport, and answers all practical requirements of block-fuel.

The present invention provides a method of utilizing raw materials or waste-products, which hitherto have been almost worthless.

The word "kneading" in the claims is intended to refer to the above described mechanical treatment to which the mixture of solid and liquid fuels is subjected.

What we claim is:—

1. The process of making fuel briquets which consists in subjecting the mixture of a solid carbonaceous combustible fuel and a liquid hydrocarbonaceous combustible fuel, to an intense mechanical working at ordinary temperatures, of such a character as to reduce in size the particles of solid fuel under treatment, and in continuing such mechanical working until the hydrocarbonaceous liquid is thoroughly incorporated in coarse, relatively dry, granular particles of crushed carbonaceous fuel so as to produce in said particles a plastic state in which they are capable of conversion into a briquet by the application of pressure merely.

2. The process of making fuel briquets which consists in mixing a solid carbonaceous combustible fuel with a liquid hydrocarbonaceous combustible fuel incapable of itself of acting as a binder for the solid fuel and subjecting the mixture to an intense mechanical kneading and crushing process at ordinary temperatures, of such a character as to reduce in size the particles of solid fuel under treatment and continuing said process until the hydrocarbonaceous liquid is thoroughly incorporated in coarse, relatively dry granular particles of the crushed carbonaceous fuel so as to produce in said particles a plastic state, and then compressing the mass into briquets.

3. In the briquetting art the process which consists in converting a solid carbonaceous fuel having the property of non-coherence with other particles of itself and a liquid hydrocarbonaceous fuel having the property of existing under ordinary conditions only in liquid form and being incapable of acting as an effective binder for the solid component, into permanently cohering binding relation by subjecting a mixture thereof to repeated intense mechanical working or kneading operations at ordinary temperatures, of such a character as to reduce in size the particles of solid fuel under treatment until the hydrocarbonaceous liquid is thoroughly incorporated in coarse, relatively dry granular particles of the crushed carbonaceous fuel so as to produce in said particles a plastic and coheringly shapable condition.

4. A fuel briquet comprising as its essential ingredient a solid carbonaceous combustible fuel and a liquid hydrocarbonaceous combustible fuel, the same being present in the form of a compressed intensely kneaded and crushed mass of the said two fuels, the hydrocarbonaceous liquid fuel being thoroughly incorporated in and carried by the crushed carbonaceous fuel.

In testimony whereof we have hereunto set our hands in presence of two subscribing witnesses.

ADRIAAN FLORIS VAN HALL.  
FEITZ BASENAU.  
RICHARD CORNELUS JOHANNUS VAN HAAGEN.

Witnesses:

CY. TIERCHS,  
T. V. A. KAKEL.